

# UNITED STATES PATENT OFFICE.

WILLIAM A. FAIRBURN, OF SHORT HILLS, NEW JERSEY, ASSIGNOR TO THE DIAMOND MATCH COMPANY, OF CHICAGO, ILLINOIS, A CORPORATION OF ILLINOIS.

## MATCH.

1,150,857.

Specification of Letters Patent. Patented Aug. 24, 1915.

No Drawing.

Application filed November 29, 1912. Serial No. 733,955.

To all whom it may concern:

Be it known that I, WILLIAM A. FAIRBURN, a citizen of the United States, and resident of Short Hills, in the county of Essex and State of New Jersey, have invented certain new and useful Improvements in Matches, of which the following is a specification.

The object of this invention is to produce a match having a splint possessing non-combustible and non-glowing characteristics, whereby when the match is ignited and the flame of the head-composition and burning substance extinguished the splint not only is devoid of spark and afterglow but its original size and shape are unimpaired. To this end, match splints are impregnated with a solution of materials which impart non-combustible, non-flaming and non-glowing properties to the splints. The match stock may first be treated with the solution and the splints be cut from the impregnated stock; or the treatment of the splints with the solution may be effected after they have been cut from non-impregnated stock. The impregnated splints are dipped into and thus permeated to the desired extent with an inflammable substance, such as molten paraffin wax, and are then headed with ignition composition in the usual manner. When the matches thus produced are ignited the fire passes through and along the splints consuming practically only the therein contained paraffin or inflammable matter without burning the body of the splints, and, as above mentioned, when the flame is extinguished the splints are devoid of spark or afterglow.

A mixture of materials which well imparts the desired non-combustible, non-flaming and non-glowing characteristics to the splints comprises, for example, ammonium acid phosphate  $(\text{NH}_4)_2\text{HPO}_4$ —500 parts and ammonium sulfate  $(\text{NH}_4)_2\text{SO}_4$ —100 parts, dissolved in water 8000 parts, preferably in the order just given. This solution is heated to about 180° Fahr., and the match splints are dipped or immersed therein for a sufficient period of time until the requisite impregnation of the splints has been effected.

It is to be understood that the described fireproofing and non-glowing properties may be imparted to the splints by materials other than those above described, without de-

parture from my invention, which, broadly considered, contemplates a match having a splint of permeable material possessing non-combustible, non-flaming and non-glowing characteristics and permeated to the desired extent with an inflammable substance, whereby when the match is ignited the fire which passes through the splint does not impair the size or shape of the splint but consumes practically only the said inflammable substance, and whereby when the flame is extinguished the splint is devoid of spark or afterglow.

What I claim is—

1. A match having a splint of permeable material with which is incorporated a substance which renders said material non-combustible, non-flaming and non-glowing throughout its length, and with which material is incorporated in addition to the first-named substance a substance which burns with flame along the non-burning body of the splint.

2. A match having a splint of permeable material possessing non-combustible, non-flaming and non-glowing characteristics and permeated to a substantial extent with an inflammable substance, whereby when the match is ignited the fire which passes through and along the splint does not impair the size or shape of the splint but consumes practically only the said inflammable substance.

3. A match having a splint of permeable material impregnated with a mixture of ammonium acid phosphate and ammonium sulfate in such proportion as to render the splint non-combustible, non-flaming, and non-glowing, and permeated to a substantial extent with an inflammable substance.

4. A match having a splint of permeable material impregnated with a mixture of ammonium acid phosphate and ammonium sulfate in such proportion as to render the splint non-combustible, non-flaming and non-glowing and permeated to a substantial extent with paraffin.

Signed at New York in the county and State of New York this 26th day of November 1912.

WILLIAM A. FAIRBURN.

Witnesses:

FRANCES R. GRIFFIN,  
B. CHANDLER SNEAD.